

# United States Patent

Bruno et al.

[15] 3,639,097

[45] Feb. 1, 1972

[54] **IMINE-TERMINATED POLYMERS  
IMPROVE COTTON DURABLE PRESS  
PRODUCTS**

[72] Inventors: **Joseph S. Bruno, Chalmette; Robert J. Harper, Jr., Metairie; John D. Reid, New Orleans, all of La.**

[73] Assignee: **The United States of America as represented by the Secretary of Agriculture**

[22] Filed: **May 13, 1969**

[21] Appl. No.: **824,252**

[52] U.S. Cl.....**8/116.2, 8/120, 8/116.3,  
8/115.6**

[51] Int. Cl.....**D06m 13/48, D06m 13/54, D06m 13/34**

[58] Field of Search .....**8/116.2, 120, 116.3**

[56] **References Cited**

UNITED STATES PATENTS

3,523,750 8/1970 **Tesoro.....8/116.2**

3,516,781 6/1970 **Pensa et al.....8/116.3**

*Primary Examiner*—George F. Lesmes

*Assistant Examiner*—J. Cannon

*Attorney*—R. Hoffman and W. Bier

[57] **ABSTRACT**

Imine-terminated polymers having polyalkylene ether moieties with a molecular weight between 500 and 10,000 have been used to improve the wet and conditioned wrinkle recovery and smooth-drying characteristics of cotton fabrics. Durable press performance can then be achieved by treatment with said polymers in combination with a less than usual amount of cross-linking agent. Such a system produces a fabric with higher conditioned and wet wrinkle recovery and better breaking strength, tearing strength, and abrasion resistance than conventional treatment. These polymers also have been used in combination with preferential cross-linking and wet fixation methods to produce fabric with improved wrinkle recovery and increased abrasion resistance.

**3 Claims, No Drawings**

IMINE-TERMINATED POLYMERS IMPROVE COTTON  
DURABLE PRESS PRODUCTS

A nonexclusive, irrevocable, royalty-free license in the invention herein described, throughout the world for all purposes of the United States Government, with the power to grant sublicenses for such purposes, is hereby granted to the Government of the United States of America.

This invention relates to the treatment of cellulosic materials with an imine-terminated polymer having a polyalkylene ether moiety. Particularly, this invention relates to an improvement of certain physical properties of cotton and other cellulosics which are treated with a cross-linking agent to produce wash-wear or durable press characteristics. More particularly, the amount of cross-linking agent required can be reduced 20-50 percent to achieve adequate wash-wear or durable press performance. The process of this invention finds utility in the fabrication of wash-wear and durable press garments.

The main object of the instant invention is to provide a new and improved method for treating cotton textiles to impart wash-wear or durable press properties to the finished garment, or the like.

A second object of the instant invention is to provide durable press garments with improved abrasion resistance.

A third object of the instant invention is to provide improved breaking and tearing strength on durable press garments.

A fourth object of the instant invention is to provide a desirable hand to cotton durable press garments.

In the prior art we find that Harper, et al. disclose in Textile Industries, May 1967 a process wherein cotton fabrics are treated with polyacrylates to impart abrasion resistance, wrinkle recovery, and breaking strength. The cotton textiles treated by the said process made the fabric stiff and unsuitable for garment use unless the polyacrylates were used with a softening agent.

where R is a poly(alkylene ether) glycol moiety, and n is equal to the number of these groups required to bring the molecular weight of this polymer to the preferred weight. For our purpose the preferred polymer is one with a molecular weight in the range of 500 to 10,000. Theoretically the cellulosic derivative would have structural formula represented thusly:



The ingredients of our formulation require no additional softeners. The cellulosic derivative produced by the process of our invention contains a built-in softener.

In the process of investigation that led to the instant invention we have learned that unlike the textile products produced by processes of the prior art the textile testing results obtained have been in many instances inverse to the expected. For example, where in the prior art the tearing and breaking strengths have been decreased as the wrinkle recovery angles have been increased, in the instant invention we have tearing and breaking strengths which have been increased as the wrinkle recovery angles have been increased. Other physical characteristics have likewise been altered by the process of the instant invention. For a closer study of these results we call attention to Table I.

TABLE I.—COTTON PRINTCLOTH TREATED WITH IMINE-TERMINATED POLYETHER AND DMEU

| Treatments        | Wrinkle recovery<br>(W+F)         |             | Elmendorf<br>tearing<br>strength<br>(W) (g.) | Breaking<br>strength<br>(W) (lb.) | Stoll flex<br>abrasion<br>(W)<br>(cycles) |
|-------------------|-----------------------------------|-------------|----------------------------------------------|-----------------------------------|-------------------------------------------|
|                   | Polymer<br>polyether <sup>1</sup> | Crosslinker | Cond.,<br>deg.                               | Wet,<br>deg.                      |                                           |
| None              | 6% DMEU                           | 274         | 246                                          | 500                               | 32.9                                      |
| 10%               | 6% DMEU                           | 315         | 301                                          | 533                               | 29.1                                      |
| 15%               | 6% DMEU                           | 317         | 306                                          | 600                               | 31.8                                      |
| 20%               | 6% DMEU                           | 317         | 311                                          | 663                               | 35.4                                      |
| Untreated control |                                   | 184         | 165                                          | 753                               | 50.1                                      |

<sup>1</sup> Polymer applied by emulsion method.

Polyurethanes were applied to cotton by Blanchard, et al., as disclosed in Textile Industries, Jan. 1967, a process which also improves the physical properties of textiles and likewise made the treated fabrics stiffer.

The problem of stiffness in this prior art has been solved by the application of softeners, such as silicones, which of course makes the process less efficient costwise and otherwise.

Now we have discovered a chemical process where the physical properties are enhanced without affecting the stiffness of the fabric. The process of the instant invention can be either a single or a two-step process. The single step process is useful for treating fabrics where the entire bath would be used, and no storage would be required for the chemicals. The two-step process would be more suitable for instances where a prepared emulsion would break upon extended storage, therefore separate storage of ingredients would be preferred.

The process of the instant invention is one involving the use of imine terminated polymers of the general formula:



It can be seen in Table I that the polyether has a pronounced effect upon both types of wrinkle recovery. Pretreatments with the polymer, followed by the application of 6 percent dimethylolethyleneurea (DMEU) produced a printcloth fabric with 315° (W+F) conditioned wrinkle recovery, approximately 40° greater than fabric treated with DMEU only. The improvement in wet wrinkle recovery ranged from 55°-65°, depending upon the level of polymer pretreatment. The maximum increase in both conditioned and wet wrinkle recovery occurs upon application of polymer without cross-linking agent to untreated fabric. In one such application by organic solvent, using 9 percent polyether in tetrachloroethylene, the conditioned wrinkle recovery was 262° (W+F) and wet wrinkle recovery of 265° representing increases of 65° and 90° respectively over the corresponding values of the untreated control. The softening action of the polymer is reflected in the improved tearing strengths of the polyether treated fabrics over the control treated with DMEU. This improvement is very high in view of the high level of conditioned wrinkle recovery achieved by the combination treatments of polymer and cross-linking agent. A tearing strength retention of 88 percent was achieved with the highest level of polymer treatment as can be seen in Table I. Also it can be seen that the fabric breaking strength improves as a function of the amount of polymer used in the treatment. In Table I the warp breaking strength of cotton printcloth treated by the

process of the instant invention increases from 29 pounds with 10 percent polymer up to 35 pounds with a 20 percent application. Although the DMEU-treated control shows a strength of 32.9 pounds, intermediate in this series, the significantly lower wrinkle recovery of the control must be deemed a compensating factor.

A comparison of the treatments with comparable wrinkle recovery performance shows (Table II) an improvement from 30 to 42 pounds in breaking strength in one case and from 30 to 38 pounds in another case from the case of the polymer additive. Even for the examples in which equal amounts of DMEU were applied to the fabric, an improvement of 6 and 8 pounds in warp breaking strength occurred.

TABLE II.—COTTON PRINTCLOTH TREATED WITH IMINE-TERMINATED POLYETHER, DMEU, AND POLYETHYLENE

| Treatments        | Crosslinker plus 1% PE <sup>2</sup> | Wrinkle recovery (W+F) |           | Elmendorf tearing strength (W) (g) | Breaking strength (W) (lb.) | Stoll flex abrasion (W) (cycles) |
|-------------------|-------------------------------------|------------------------|-----------|------------------------------------|-----------------------------|----------------------------------|
|                   |                                     | Cond., deg.            | Wet, deg. |                                    |                             |                                  |
| None              | 2% DMEU                             | 258                    | 222       | 787                                | 36                          | 882                              |
| 7%                | 2% DMEU                             | 290                    | 286       | 813                                | 42                          | 1728                             |
| None              | 4% DMEU                             | 287                    | 244       | 660                                | 30                          | 314                              |
| 7%                | 4% DMEU                             | 304                    | 303       | 673                                | 38                          | 1337                             |
| None              | 6% DMEU                             | 302                    | 262       | 573                                | 30                          | 124                              |
| Untreated control |                                     | 197                    | 173       | 1053                               | 51                          | 1139                             |

<sup>1</sup> Applied dissolved in perchloroethylene.

<sup>2</sup> Polyethylene.

In Table I it may be observed that with increasing amounts of the polyether add-on the Stoll flex abrasion resistance improves progressively until it is approximately 95 percent of that of untreated cotton. This occurs in fabric with conditioned and wet recovery angles above 310° and with a high level of cross-linking agent (6 percent DMEU). With the lower levels of cross-linking agent reported in Table II, the polymer treated samples still have approximately 290°-310° conditioned wrinkle recovery and Stoll abrasion resistance greater than that of the untreated cotton.

Although Tables I and II illustrate the invention as reduced to practice employing dimethylolethyleneurea (DMEU), for our purpose the process of the instant invention is applicable to other cross-linking agents. We have found that any acid catalyzed cross-linking agent can be used in place of the DMEU.

#### EXAMPLE 1

##### POLYETHER EMULSION TWO-BATH PROCESS

An emulsion was formulated and the imine-terminated polymer having a polyalkylene moiety was dissolved in an organic solvent, then emulsified, was prepared containing the indicated quantities of the selected ingredients.

| Ingredient                                     | Quantity (% of bath, by wt.) |
|------------------------------------------------|------------------------------|
| Polyalkylene ether                             | 10                           |
| Mineral spirits                                | 10                           |
| Emulsifying agent (Monostearate, Atlas G-2162) | 3                            |
| Water                                          | 77                           |

A cross-linking solution which would be suitable for cross-linking of the cellulose structure of cotton was prepared, containing a computed quantity of an acid-type catalyst, as follows:

| Cross-linking agent                                  | Quantity (% of bath, by wt.) |
|------------------------------------------------------|------------------------------|
| Dimethylolethylene urea                              | 6.0                          |
| Zn(NO <sub>3</sub> ) <sub>2</sub> ·6H <sub>2</sub> O | 0.4                          |
| Water                                                | 93.6                         |

The emulsion was applied to a sample of 80×80 cotton printcloth by padding with standard techniques to a wet pickup of about 80 percent, dried 10 minutes at 60° C. (the sample had a dry add-on of 8.0 percent), and then the solution containing the cross-linking agent and catalyst were applied to a wet pickup of about 80 percent. The fabric sample was then mounted on a pin frame to maintain the original dimensions of the untreated sample. The impregnated sample was then dried 7 minutes at 60° C., then cured 3 minutes at 160° C.

10 The finished sample was submitted to a selected group of textile tests. The significant improvements found among these are listed below in a comparative study. The treated sample had a weight gain of 8.5 percent.

| 30                                  | Sample 1 Tests | Sample 1 | Results   |
|-------------------------------------|----------------|----------|-----------|
| 35                                  |                |          | — Control |
| Elmendorf Tearing Strength          | 533            | g.       | 500       |
| Breaking Strength                   | 133.4          | lbs.     | 32.9      |
| Stoll Flex Abrasion                 | 284            | cycles   | 268       |
| Wrinkle Recovery (conditioned, W+F) | 315            | degrees  | 274       |

In reference to the physical testing methods it should be pointed out that the Elmendorf Tearing Test carries an ASTM Designation of Method D1424-63; the Breaking Strength Test Designation is Method 1682-64; the Stoll Flex Abrasion Designation is Method D1175-64T; and the Wrinkle Recovery Test Designation is 1295-60T; these designations by the American Society for Testing and Materials, Philadelphia, Pa.

#### Example 2

##### A TWO BATH SOLVENT PROCESS

50 The imine-terminated polymer having a polyalkylene moiety was dissolved in a selected organic solvent, the bath contained the indicated quantities of the selected ingredients.

| 55 | Ingredient                                      | Quantity (% by wt.) |
|----|-------------------------------------------------|---------------------|
|    | Imine-terminated polyether<br>Perchloroethylene | 7<br>93             |

60 A second solution was prepared, this contained the cross-linking agent, the selected catalyst, and water. The formulation was prepared thusly:

| 65 | Cross-linking agent                                  | Quantity (% by wt.) |
|----|------------------------------------------------------|---------------------|
|    | Dimethylolethylene urea                              | 4.0                 |
|    | Zn(NO <sub>3</sub> ) <sub>2</sub> ·6H <sub>2</sub> O | 0.4                 |
|    | Water                                                | 95.6                |

70 Application from organic solvents has been contemplated for modern textile plants which are capable of using organic solvents for processing textiles. For this reason, this particular sample was handled in this manner.

75 The first solution was applied to a cotton printcloth in conventional equipment but equipped with well-ventilated

devices. The excess solution was removed to obtain a wet pickup of 120 percent. The wet impregnated textile was dried 7 minutes at 60° C., and the equilibrated textile was found to have gained 8.5 percent in weight.

The treated dry sample was then impregnated with the second solution, which contained the cross-linking agent and catalyst. The wet pickup obtained was 80 percent. The textile was then dried 7 minutes at 60° C., and cured 3 minutes at 160° C. The fabric sample was then water washed and allowed to dry. The weight gain computed from the untreated original weight of the sample was labeled as "total weight gain: 10 percent."

The significant results of textile testing were selected as before, and are here tabulated.

| Sample 2<br>Tests                             | Sample 2 | Results | Control |
|-----------------------------------------------|----------|---------|---------|
| Elmendorf Tearing Strength                    | 813      | g.      | 787     |
| Breaking Strength                             | 42       | lbs.    | 36      |
| Stoll Flex Abrasion                           | 1,728    | cycles  | 882     |
| Conditioned Wrinkle Recovery (warp + filling) | 290      | degrees | 258     |

### EXAMPLE 3

#### A SINGLE-BATH EMULSION PROCESS

The imine-terminated polymer was formulated so as to include the cross-linking agent, a selected catalyst, a wetting agent, an organic solvent, an emulsion stabilizer, and water, all in the same bath. The bath contained the indicated quantities of the selected ingredients.

| Ingredient                                           | Quantity(% by wt.) |
|------------------------------------------------------|--------------------|
| Dimethylolethylene urea                              | 5.0                |
| Zn(NO <sub>3</sub> ) <sub>2</sub> ·6H <sub>2</sub> O | 0.5                |
| Emulsifying agent                                    | 3.0                |
| (Monostearate, Atlas G-2162)                         |                    |
| Stabilizing agent                                    | 4.0                |
| (Ester Phosphate, Victamul 89)                       |                    |
| Wetting agent (Polyether sulfate, Triton X-100)      | 0.1                |
| Polyether                                            | 13.0               |
| Benzene                                              | 13.0               |
| Water                                                | 61.4               |

### EXAMPLE 4

#### INCORPORATING WITH WET-FIXATION

To illustrate another embodiment of the instant invention an imine-terminated polymer of the instant invention was used to supplement a "wet-fixation process" described by Hollies and Getchell in Textile Research J., Vol. 37, pp. 70-76 (1967). The adaptation can be made to other known "wet-fixation processes" as well.

"Fixed" samples were provided by a commercial textile mill using the Hollies and Getchell procedure. These samples were further processed by applying the imine-terminated polyether of our invention. Results of comparative study are shown in table III.

Wet fixation is a method of internal polymer deposition in which the fiber remains somewhat swollen during the polymer deposition step. The resultant fabric generally has good abrasion resistance, but wrinkle recovery values obtained from mill finished fabric are frequently low. The imine-terminated polymer improves the performance of wet-fixed fabrics in that lower than normal wrinkle recovery angle can be raised to durable press performance.

A single bath emulsion formulation was prepared thusly:

| Ingredient                       | Quantity(% by wt.) |
|----------------------------------|--------------------|
| Imine-terminated polyether       | 17.0               |
| Benzene                          | 17.0               |
| Monostearate (emulsifying agent) | 4.0                |

|                                                                 |      |
|-----------------------------------------------------------------|------|
| Zn(NO <sub>3</sub> ) <sub>2</sub> ·6H <sub>2</sub> O (catalyst) | 0.4  |
| Water                                                           | 61.6 |

5 The emulsion was then padded onto the uncured wet-fixed sample to a wet pickup of 80 percent, dried at 60° C. for 7 minutes and cured at 160° C. for 3 minutes. A comparison of selected tests for the standard wet fix process and the wet fix process modified with the polyalkylene ether polymer is indicated in table III.

TABLE III.—APPLICATION OF IMINE-TERMINATED POLYETHER TO WET FIXED CORDUROY

| 15 |                                                                    | Wrinkle recovery |              | Fill<br>tear<br>(g.) | Fill<br>break<br>(lb.) | Stoll flex<br>abrasion<br>(cycles) |
|----|--------------------------------------------------------------------|------------------|--------------|----------------------|------------------------|------------------------------------|
|    |                                                                    | Cond.,<br>deg.   | Wet,<br>deg. |                      |                        |                                    |
|    | Uncured wet fixed fabric                                           | 168              | 190          | 783                  | 45.8                   | 467                                |
|    | Cured wet fixed fabric                                             | 236              | 211          | 417                  | 29.0                   | 200                                |
| 20 | 17% polyether <sup>1</sup> pre-treated then cured wet fixed fabric | 316              | 289          | 600                  | 34.3                   | 1,533                              |

<sup>1</sup> Polymer applied from emulsion.

### EXAMPLE 5

#### BACK-COATING WITH THE CROSS-LINKING AGENT

An imine-terminated polymer containing formulation was prepared for the first bath, containing the indicated quantities of the selected ingredients.

| Ingredient                                           | Quantity(% by wt.) |
|------------------------------------------------------|--------------------|
| Imine-terminated polyether                           | 10.0               |
| Benzene                                              | 10.0               |
| Emulsifying agent                                    | 4.0                |
| Zn(NO <sub>3</sub> ) <sub>2</sub> ·6H <sub>2</sub> O | 0.4                |
| Water                                                | 75.6               |

40 The emulsion was then applied to a sample of 6 oz. cotton sateen, dried 7 minutes at 60° C., and weighed.

The dried impregnated textile was then given a back coating by the process described by Cooper et al. in the American Dyestuff Reporter, Vol. 54, page 89 (1965), using an aqueous formulation containing 0.8 percent hydroxyethylcellulose (thickener) and 12 percent dimethylolpropyleneurea. This was applied to the back of the fabric to obtain a 30 percent wet pickup with a knifeblade center.

45 A sateen cuff was prepared from this sample, and this was submitted to a standard laundry testing procedure. The cuff thus prepared was submitted to 20 standard laundering cycles, and was found to have lasted 18 cycles before minor abrasion damage was noted. The wrinkle recovery angle (warp plus filling) after the 20 laundering cycles was a suitable 260° C.

50 NOTE: When a sateen cuff was prepared as in example 5, above, but increasing the dimethylolpropylene urea content to 15 percent and excluding the imine-terminated polyether of this invention the results obtained were significantly unsatisfactory. The wrinkle recovery angle evaluation was 243° after 20 laundering cycles, and minor damage was noted at the end of the 9th cycle. Improved wrinkle recovery and abrasion resistance were imparted by the use of imine-terminated polyether of the instant invention.

We claim:

1. A process for imparting to a cotton cellulosic textile which has been wet-fixed with an aminoplast resin the desirable qualities obtained in cross-linking the cellulose but without the wrinkle recovery losses generally associated with such treatments, comprising:
  - a. impregnating the dried, wet-fixed cotton cellulosic textile with a single bath emulsion containing about 17 percent benzene, about 4 percent monostearate emulsifying agent, about 0.4 percent of an acid catalyst selected from the group consisting of zinc nitrate hexahydrate catalyst and magnesium chloride hexahydrate, about 61.6 percent water, and about 17 percent of an imine-terminated polymer having the formula



wherein R is a poly(alkylene ether) glycol moiety and n is equal to the number of these groups required to bring the

molecular weight of the polymer to about from 500 to 10,000 to obtain a wet pickup of about 80 percent;

- b. drying the impregnated textile for about 7 minutes at about 60° C.; and
- c. curing the dried, impregnated textile for about 3 minutes at about 160° C.

2. The process of claim 1 wherein the catalyst is zinc nitrate hexahydrate.

3. The process of claim 1 wherein the catalyst is magnesium chloride hexahydrate.

\* \* \* \* \*

15

20

25

30

35

40

45

50

55

60

65

70

75